

## UNITED STATES PATENT OFFICE

2,021,849

VISCOSE AND CUPRAMMONIUM CELLULOSE  
SPINNING SOLUTIONS AND PRODUCTS  
THEREOFRudolph S. Bley, Elizabethton, Tenn., assignor to  
North American Rayon Corporation, New  
York, N. Y., a corporation of DelawareNo Drawing. Application September 8, 1934,  
Serial No. 743,301

## 10 Claims. (Cl. 106—40)

The present invention relates to the production of soft-lustre cellulosic products, such as filaments, yarns, ribbons, films, etc., from viscose and cuprammonium cellulose solutions.

One object of my invention has to do with the emulsification of an alkyl-naphthalene—having the structure  $C_{10}H_7.(R)_x$  in which R represents an alkyl group—with a cellulosic spinning solution to produce, after extrusion into conventional spinning baths, soft-lustre products of pleasing hand.

Another object of my invention relates to the incorporation of a phenyl-naphthalene—having the structure  $C_{10}H_7.(R_1)_x$  in which  $R_1$  represents a phenyl group—into cellulosic spinning solutions for the manufacture of soft-lustre products.

Other objects of my invention will become apparent to those skilled in the art after a study of the following specification.

I am well aware that it has, heretofore, been proposed to disperse hydronaphthalenes and halogenated naphthalenes in cellulosic spinning solutions with a view of obtaining delustered filaments. However, it has been found that hydronaphthalenes evaporate too rapidly from the extruded filaments, and that halogenated naphthalenes, such as Halowax, are rather unstable in combination with cellulosic products, this being probably due to their chlorine content. These deficiencies, however, are unexpectedly overcome by uniformly distributing and/or emulsifying high-boiling alkyl- and phenyl naphthalenes in viscose and cuprammonium cellulose solutions. The following table will serve to illustrate the physical characteristics of some naphthalene derivatives suitable as delustering agents, although I wish to emphasize that my process is not limited to these compounds. Any alkyl- and phenyl-derivative of naphthalene, which is substantially water- and alkali-insoluble, colorless and resistant to the attack by acidic spinning baths, may be used to modify the lustre of viscose and cuprammonium cellulose products. In order to prevent rapid evaporation from the extruded products, I prefer to use alkyl- and phenyl-naphthalenes boiling above 100° C. The amounts of these derivatives may be varied within wide limits, although an addition of about 1 to 10% is generally sufficient to deluster the aforementioned cellulosic products, these percentages being calculated on the cellulose content of the solutions.

After thoroughly emulsifying the naphthalene derivative with the spinning solution, it is spun in conventional manner into setting baths. Finely divided pigments, such as titanium dioxide, etc.,

may be dispersed in an alkyl- or phenyl-naphthalene to form an organosol. Subsequently this organosol may be emulsified with a spinning solution to modify the lustre of the finished products.

I wish to emphasize that the compounds as well as the proportions, set forth above, may be varied to a large extent without departing from the spirit and scope of my invention.

TABLE 1  
Physical characteristics of some alkyl- and phenyl-naphthalenes

| Derivative                  | Boiling point<br>in centigrades | Solubility in<br>water |
|-----------------------------|---------------------------------|------------------------|
| Alpha-methyl-naphthalene    | 243                             | Insoluble.             |
| Beta-methyl-naphthalene     | 245                             | Do.                    |
| Alpha-dimethyl-naphthalene  | 264.3                           | Do.                    |
| Beta-dimethyl-naphthalene   | 266                             | Do.                    |
| Alpha-ethyl-naphthalene     | 258                             | Do.                    |
| Beta-ethyl-naphthalene      | 251                             | Do.                    |
| Alpha-n-propyl-naphthalene  | 274                             | Do.                    |
| Beta-n-propyl-naphthalene   | 278                             | Do.                    |
| Alpha-n-butyl-naphthalene   | 282                             | Do.                    |
| Beta-n-butyl-naphthalene    | 284                             | Do.                    |
| Alpha-iso-butyl-naphthalene | 197                             | Do.                    |
| Beta-iso-butyl-naphthalene  | 112                             | Do.                    |
| Alpha-phenyl-naphthalene    | 325                             | Do.                    |
| Beta-phenyl-naphthalene     | 345                             | Do.                    |
| Etc.                        |                                 |                        |

## I claim:

1. A spinning solution for the manufacture of soft-lustre products comprising a solution of the group consisting of viscose and cuprammonium cellulose and an ethyl-naphthalene.

2. A spinning solution for the manufacture of soft-lustre products comprising a solution of the group consisting of viscose and cuprammonium cellulose and about 1 to 10% of an ethyl-naphthalene, said percentages being calculated on the cellulose content of said solution.

3. A soft-lustre cellulosic product of the group consisting of viscose and cuprammonium cellulose containing an alkyl-naphthalene.

4. A spinning solution for the manufacture of soft-lustre products comprising a solution of the group consisting of viscose and cuprammonium cellulose and an alkyl-naphthalene, said naphthalene being substantially water- and alkali-insoluble, having a boiling point above 100° C. and the structure  $C_{10}H_7.(R)_x$  in which R represents an alkyl group.

5. A spinning solution for the manufacture of soft-lustre products comprising a solution of the group consisting of viscose and cuprammonium cellulose and a dialkyl-naphthalene, said naphthalene being substantially water- and alkali-in-

soluble and having a boiling point above 100° C.

6. A spinning solution for the manufacture of soft-lustre products comprising a solution of the group consisting of viscose and cuprammonium cellulose and about 1 to 10% of an alkyl-naphthalene, said naphthalene being substantially water- and alkali-insoluble, having a boiling point above 100° C. and the structure  $C_{10}H_7.(R)_x$  in which R represents an alkyl group and said percentages being calculated on the cellulose content of the solution.

7. A spinning solution for the manufacture of soft-lustre products comprising a solution of the group consisting of viscose and cuprammonium cellulose and about 1 to 10% of a dialkyl-naph-

thalene, said naphthalene being substantially water- and alkali-insoluble and having a boiling point above 100° C. and said percentages being calculated on the cellulose content of the solution.

8. A soft-lustre cellulosic product of the group consisting of viscose and cuprammonium cellulose containing a dialkyl-naphthalene.

9. A soft-lustre cellulosic product of the group consisting of viscose and cuprammonium cellulose containing an ethyl-naphthalene.

10. A soft-lustre cellulosic product of the group consisting of viscose and cuprammonium cellulose containing a butyl-naphthalene.

RUDOLPH S. BLEY. 15